

# United States Patent

Merker et al.

[15] 3,655,532

[45] Apr. 11, 1972

[54] **METHOD FOR ELECTROPLATING NICKEL**

[72] Inventors: **Reuven Merker**, Englewood Cliffs; **Salvatore Lucca**, Paramus, both of N.J.

[73] Assignee: **The Metalux Corporation**, Paterson, N.J.

[22] Filed: **May 6, 1970**

[21] Appl. No.: **35,225**

[52] U.S. Cl..... 204/49

[51] Int. Cl..... C23b 5/08, C23b 5/46

[58] Field of Search..... 204/49

[56] **References Cited**

UNITED STATES PATENTS

|           |         |                   |        |
|-----------|---------|-------------------|--------|
| 3,152,975 | 10/1964 | Kardos et al..... | 204/49 |
| 3,220,940 | 11/1965 | Brown et al.....  | 204/49 |
| 3,386,897 | 6/1968  | Ostrow et al..... | 204/49 |
| 3,399,123 | 8/1968  | Passal .....      | 204/49 |

FOREIGN PATENTS OR APPLICATIONS

1,164,192 2/1964 Germany ..... 204/49

Primary Examiner—F. C. Edmundson

Attorney—Clario Ceccon

[57] **ABSTRACT**

Method for electroplating nickel to obtain a bright deposit by adding to a conventional nickel acidic bath solution effective amounts of a brightening agent having the general formula



where R is a phenyl, alkyl or alkenyl radical with one to 14 carbon atoms, Y is hydrogen or an alkyl radical with one to six carbon atoms, n is a numeral from one to six, and Z is a metal imparting water solubility to the brightening agent.

**5 Claims, No Drawings**

## METHOD FOR ELECTROPLATING NICKEL

## FIELD OF THE INVENTION

The present invention is directed to a process of plating nickel from acidic bath solutions, and more particularly, to the production of bright nickel platings having improved characteristics.

## THE PRIOR ART

The use of sulfonamides and sulfonimides as primary or carrier type brighteners has long been known in the art. These brighteners have also proven capable of promoting the production of low stress ductile deposits when present in a sufficiently high concentration. They have been employed alone or in conjunction with secondary addition agents which increased the brightness and, in many cases, the leveling characteristics of the nickel bath.

One known brightener has been saccharin, the sodium salt of benzene sulfonimide or NaO-sulfobenzoic imide. Because of its solubility in water, it not only offered a means of securing a high concentration thereof in the plating bath, but also a convenient method of making additions to the plating bath. Since saccharin has a high degree of solubility, it became possible to make a concentrated solution and conveniently add it to the bath. When it is used in a Watts bath with acetylenic compounds (such as 2-butyne, 1-4 diol), it is also an effective haze remover. On the other hand, other sulfonamides, such as benzene sulfonamide tend to produce hazy or cloudy deposits with the acetylenic compounds. These hazy deposits may be corrected only by the addition of a sulfonic acid, such as benzene sulfonic acid.

Saccharin has the most undesirable characteristic of producing poor, dark, low current density deposits when the bath is contaminated with zinc or copper. Such contamination is quite common when plating zinc die castings commercially.

Benzene sulfonamide or its sodium salt when used in nickel plating baths acts similarly to saccharin as a stress reducer. However, it has limited solubility making it difficult to dissolve in the bath. Also, where relatively high concentration of the sulfonamide are required to carrying the secondary brighteners or for greater stress reduction, the limited solubility thereof limits its use. When used in conjunction with acetylenic secondary brighteners, it has a tendency to produce hazy deposits and it requires the addition of an aryl sulfonic acid such as benzene sodium sulfonate.

The halogen substituted derivatives of the sulfonamides and imides produce better leveled deposits than the unsubstituted compounds; however, they have poorer solubility. As a result, it becomes impossible to secure the optimum concentration thereof in the plating bath.

The sulfonamides and sulfonimides have decreased solubility at low pH values and, where low stressed deposits are required in nickel plating baths at pH of 1-2, it becomes impossible to secure sufficient beneficial concentration in solution.

One method of solubilizing the brightener employed in the bath solution is described in U.S. Pat. No. 3,386,897 to Ostrow. According to this patentee, the solubilization is obtained by introducing in the conventional acidic nickel plating bath an organic compound which contains both at least a sulfonamide group and at least a sulfonic acid group.

## BRIEF SUMMARY OF THE INVENTION

The present invention is intended to overcome the defects and disadvantages inherent in many prior paths of the character described above and to obtain results equal, if not superior, to those of Ostrow's, by providing a nickel plating process which will result in soft, ductile and adherent deposits on the basis metal, and haze-free over a broad current density range, particularly when acetylenic compounds are used as secondary brighteners.

It is further among the objects of the invention to provide a bath in which the additives have high solubility, give good

tolerance to impurities in the bath, such as copper, zinc, lead, etc., and which promote leveling in the deposit.

It is still further among the objects of the invention to provide a bath which contains addition agents which retain their solubilities at low pH values of the order of 1-2.

## DESCRIPTION OF THE INVENTION

In practicing the invention, there is introduced into the usual acid nickel plating bath, an organic primary brightener which contains both at least one sulfonamide group and at least one ethoxy group. The present brighteners are applicable to baths in which practically all of the known secondary brighteners are incorporated. These brighteners may be designated as ethoxylated benzene sulfonamides. They have unusually high water solubility and they impart exceptional zinc and copper tolerance to the nickel bath. They impart bright haze-free deposits when used with secondary acetylenic addition agents.

This class of brightening agent may be used alone where maximum luster and leveling are not required. They may be used in conjunction with other known primary or secondary brighteners such as acetylenic alcohols, acetylenic glycols and polyglycols, acetylenic amines and polyamines, quaternary pyridinium and quinoline compounds, allyl alcohols and amines, vinyl pyridine, triphenyl methane derivatives, aromatic sulfonic (mono and poly) acid salts.

The new compounds may be designated by the following general formula:



wherein R is a radical taken from the class consisting of phenyl, naphthyl, alkyl, alkenyl and alkynyl, having from one to 14 carbon atoms; n is a numeral from one to six; Z is a radical taken from the class consisting of hydrogen and a metal imparting water solubility to said agent; and Y is a radical taken from the class consisting of hydrogen and alkyl having one-six carbon atoms. These radicals may have substituents which do not adversely affect the desired properties of the compounds.

Among the advantages of the additives is the high solubility even at low pH values, being about 200 to 500 grams per liter compared to 1 to 3 grams per liter of the benzene sulfonamide or 200 to 400 grams of the sulfonamic-sulfonic acid mixture. This allows the production, shipment and storage of concentrated solutions with substantial savings. It permits the introduction into the bath of say 0.05 gram per liter to saturation, preferably up to 50 grams per liter. Even when chlorinated to obtain improved leveling, the solubilities of the present additives are in the neighborhood of 100 grams per liter. It is advantageous to add these brighteners to the bath in the form of concentrated solutions, both for accuracy and convenience. The alkene and alkyne derivatives give improved results. The brighteners are suitable for use in various acid nickel plating baths, including those containing sulfonates. Freedom from haze is obtained.

R may also be alkyl, alkene, and alkyne radicals having substituents thereon which do not adversely affect their properties. Aromatic radicals may be polynuclear, and have such substituents thereon such as alkyl, sulfo, halo, nitrilo, sulfoalkyl, amino and halo alkyl groups. Z may be, for instance, sodium, potassium, hydrogen, magnesium, cobalt, nickel and others.

Typical brightening agents suitable for the process of the invention are: benzene-sulfon-mono-ethoxy-amide, p-toluene benzene-sulfon-di-ethoxy-amide, p-bromo-benzene-sulfon-tri-ethoxy-amide, benzene meta-di-sulfon-tri-ethoxy-amide, alpha-naphthalene sulfon-di-ethoxy-amide, beta-naphthalene sulfon-di-ethoxy-amide, allyl-sulfon-di-ethoxy-amide, o-benzoic-sulfon-di-ethoxy-amide, p-toluene sulfon-mono-chloro-di-ethoxy-amide.

All of these compounds may be employed in the Watts bath solution given hereinafter, in various quantities ranging up to saturation, and in every instant a bright deposit may be obtained.

